

## UNITED STATES PATENT OFFICE

2,597,378

THERMOADHESIVE COMPOSITION AND  
COMPOSITE CLOSURE LINER FORMED  
THEREWITH

Louis F. Rogers and Michael S. Ebert, Wilmington, Del., assignors to Continental Can Company, Inc., New York, N. Y., a corporation of New York

No Drawing. Application May 8, 1946,  
Serial No. 668,310

2 Claims. (Cl. 260—28.5)

1

It has been a practice in making closures having cushioned liners; for example, in crown seals for bottles, etc., to have a cork cushion cemented to the metal shell, and the bottle, etc., orifice is closed by a liner or spot which is secured to the cushion by a gutta percha cement.

According to the present invention, a superior article is produced by securing the spot to the cushion by a cement consisting essentially of a mixture of butyl rubber and paraffin; the characteristics of such mixture giving benefit to its use under conditions of hot application and under conditions where a strong and self-healing cement film is desired for making such closure liners and in other cases where repeated transition from tacky adhesiveness to non-tacky adhesiveness is desired.

Butyl rubber is an article of commerce, being produced in known ways from petroleum hydrocarbons by low-temperature catalytic polymerizing combinations of isobutylene with butadiene or, preferably, isoprene, and having characteristics resembling those of natural rubber but differing therefrom in its behavior in the presence of petroleum oils and waxes or more facile mixing and the exhibition of superior conditions of adhesiveness when admixed therewith.

As an example of practice, 10 pounds of commercial butyl rubber (GR-I-60) was mixed, on a rubber mill at room temperature, with 10 pounds of ordinary paraffin wax until a uniform product results. This material was heated to about 250 degrees F., becoming quite fluid, and was applied to a base consisting of aluminum foil of the grade and thickness employed for crown seal spots, and was spread and worked into a film having a thickness of about 0.002 to 0.003 inch, and then cooled to fix it in place. Hot roller coating or doctor blade apparatus can be used; for small surfaces, a plate or spatula can be employed. The mixture is plastic and adherent to the sheet at 200 degrees F. and will harden to increased strength and tightly adherent condition when left at 100 to 120 degrees F. or below, so that the coated film can then be handled and is essentially free of tackiness at normal room temperatures.

When the base and its coating is not to be immediately used, as is the normal case in placing spots in crown seals, it is preferable to roll the cooled composite into a coil for storage and shipment. When the material is compounded for a very low softening or tacky temperature, a glassine or cloth interleaf may be used. The spotting machine then receives such a roll and unwinds it, while stripping the interleaf away if

2

such be used, and advancing the laminar web of foil and coating through the devices for punching the spots and applying them to the cushions of the crown seals under heated conditions whereby the said mixture is again made tacky and thereby adherent to the cushions.

The fusion, tacky, and hardening temperatures for the mixture can be controlled by proportioning. Thus, a desirable and effective range of properties can be attained by relative proportions by weight of butyl rubber : paraffin wax of substantially 50:50 to 60:40. Contents of butyl rubber much less than 50 percent are usually too low in tensile strength and hardening temperature to permit easy employment in the spotting machines, due to premature softening and tackiness under the hot conditions of operating the machines, and also have a reduced adhesiveness: while a content of 70 percent or over of butyl rubber leads to mixtures which do not exhibit the necessary tackiness, adhesiveness and thermoplasticity to provide adequate cementing layers. Within these ranges, the butyl rubber and paraffin are fully compatible and miscible with one another to provide uniform and stable mixtures.

The stability of the mixture as made and as employed in coating metal, vinyl resin, chlorinated rubber, varnished paper, etc., webs and sheets, or other articles, such as the aluminum foil used above for the spots, is striking in comparison with apparent equivalents. Thus, mixtures of paraffin wax with natural or buna rubbers, latex, etc., have a shelf life of a few days, after which the mixture is not competent of producing a tacky surface upon the normal heating or does not upon later cooling afford a strong and permanent bond. Some of the synthetic rubbers, such as chlorinated butadiene elastomers, reject paraffin or petroleum wax and give no tacky product at all. On the contrary, the present mixtures can be subjected to repeated cycles of heating to tackiness or fusion and then of cooling to surface hardness, without losing the desirable properties of thermo-adhesiveness upon heating and strength while cooled to 32 degrees F. and below.

The other forms of butyl rubber in commerce can be used; for example, mixtures with GR-I-40 are more tacky at any given temperature than those with GR-I-60, but are less viscous at room temperatures so that they may be extruded from between a foil spot and the cushion, while capping a bottle of warm liquid, and thus cause undesirable adhesion between the glass and cork

outside the area of the spot, but this very characteristic is of value where such adhesion is sought as a means of providing a secondary liquid and moisture-proof seal at such point. Butyl rubber has been defined by trade specifications such as those of the "Committee on Specifications for Synthetic Rubbers" of Rubber Reserve Company. GR-I is a standard product having a Mooney viscosity value between 40 and 50. Special grades are available: thus, GR-I-40 has a Mooney viscosity between 30 and 40, while GR-I-60 has a Mooney viscosity between 50 and 60. It is preferred to employ butyl rubber having a viscosity within the limits of substantially 30 to 70. Low viscosities have lower strength, while high viscosities are hard to work.

The preferred wax is a fully refined paraffin wax of about 132-135 degrees F. (American Melting Point), a specific gravity at 60 degrees F. (solid) of 0.889 and essentially of crystalline structure as distinguished from microcrystalline structure: and is available in commerce under such designation. The commercial product known as "Atlantic Refining Company No. 171" has been found useful. The same company's "No. 191" with a melting point of about 138-140 degrees F. is also satisfactory, while requiring a slightly higher temperature in use. These give a product which is non-tacky at normal room temperatures, and has a relatively sharp softening point so that the mass loses its tackiness rapidly during its cooling from high temperature, and thus quickly produces a stable bond. In general, the paraffin should be waxy at room temperature (e. g. 80 degrees F.); should soften at a temperature well below that at which the butyl rubber is damaged, preferably below a temperature of around 150 degrees F. so that water bath or low steam pressure conditions can be employed in spreading the mixture; should be well compatible with the butyl rubber; and preferably should be of comparatively high tensile strength (e. g. "Atlantic No. 171" has a tensile strength of 300 p. s. i.).

It is at times desirable to add a material to reduce the surface-tack of the cooled material and to improve the adhesion effected while hot: that is, to prevent adhesion by the exposed surface of the mixture after the latter has been applied to foil and cooled, so that the turns of the wound coil will not stick together or block while it is being unwound during employment. An addition up to 10 percent of a non-heat-hardening resin compatible with the butyl rubber and the paraffin, such as thermoplastic hydrocarbon resins of the olefin, diolefin, cyclopentadiene, styrene, and cumarone-indene types, having long aliphatic chains, is effective for this. A presently preferred resin, when such addition is desired, is a mixture of polymers having a wide range of molecular weights and produced from crude mixtures of styrene and styrene homologs such as those obtained from the fractionation of so-called "Crude Solvent" from the light oils scrubbed out of coke oven or gas house gas; specifically, a useful mixture of such polymers is a soft solid at room temperature and demonstrates a slick waxy feeling at the undisturbed surface at room temperature, but exhibits stickiness when the mass is disturbed. This preferred styrene resin mixture is permanently thermoplastic, melts with essential sharpness at about 50 degrees C., and is heat-stable up to 175 degrees C. or above. It is compatible up to equal parts with paraffin wax and oil and in essentially

any proportion with the rubber. These styrene resins are commercially available, and the material sold as "Piccolastic A-50" is satisfactory. This effect can also be gained by including up to a like percentage of natural rubber, which leads to a slight surface oxidation that acts to prevent blocking.

A general characteristic of the adhesive is that it remains essentially non-tacky for a long time provided that it is kept at below about 80 degrees F., and can be utilized by simple heating, being self-healing under such conditions; spots of foil having the adhesive thereon can be applied to cork cushions and primary adhesion obtained by low heating before further heating to essential fusion is used to seal and assure maximum strength. The self-healing and tasteless behavior assures that the seal will be essentially maintained during the minor distortions and weakenings of the foil produced during the capping operations.

The shelf life of the mixture permits the coating of film at a central plant and its shipment under ordinary temperature conditions to the spotting plant; and the storage of a large stockpile of coated film.

The aluminum foil is an illustrative example of a film material of limited permeability for liquids and vapors, and the composition cork disk is an example of a cellulosic cushion material. Obviously, as indicated, other materials may be substituted as a base, and such materials adhered to metal, or to the cellulosic surfaces of cork, paper, wood, etc., by the heating operations.

It is obvious that the invention is not restricted to the illustrative forms of practice, but that the same may be employed in many ways within the scope of the appended claims.

What is claimed is:

1. A composition capable of exhibiting tackiness upon each heating during repeated cycles of heating above and cooling below room temperature, and having the property of strong adhesion to metal and cellulosic surfaces after cooling in contact therewith, consisting of 40 to 50 parts by weight of paraffin wax having a melting point between 80 and 150 degrees F., and 60 to 50 parts by weight of a butyl rubber produced by low-temperature catalytic polymerizing combination of isobutylene with a substance selected from the group consisting of butadiene and isoprene, said butyl rubber having a Mooney viscosity of 30 to 70, the said ingredients being intimately and uniformly mixed.

2. A closure liner material comprising a film of material of limited permeability and on a face thereof a thermo-adhesive coating of a cement consisting of 40 to 50 parts by weight of paraffin wax with a softening point of substantially 132 to 135 degrees F., and 60 to 50 parts by weight of a butyl rubber produced by low-temperature catalytic polymerizing combination of isobutylene with a substance selected from the group consisting of butadiene and isoprene, said butyl rubber having a Mooney viscosity of 30 to 70, the said ingredients being intimately and uniformly mixed, said coating having a thickness of substantially three to four thousandths of an inch.

LOUIS F. ROGERS.  
MICHAEL S. EBERT.

## REFERENCES CITED

The following references are of record in the file of this patent:

## UNITED STATES PATENTS

| Number    | Name          | Date          |
|-----------|---------------|---------------|
| 2,227,516 | Soanes        | Jan. 17, 1941 |
| 2,275,814 | Abrams et al. | Mar. 10, 1942 |
| 2,367,250 | Warth et al.  | Jan. 16, 1945 |
| 2,403,964 | Bannon        | July 16, 1946 |
| 2,413,239 | Mason         | Dec. 24, 1946 |
| 2,419,304 | Warth et al.  | Apr. 22, 1947 |

5

## FOREIGN PATENTS

| Number  | Country   | Date          |
|---------|-----------|---------------|
| 112,875 | Australia | Apr. 24, 1941 |

## OTHER REFERENCES

Page 1, Butyl Rubber, a publication of Stanco Distributors, Inc., 26 Broadway, New York, New York. Received in Pat. Off. Lib. December 1942. India Rubber World, June 1943, page 269.

10